

## UNITED STATES PATENT OFFICE

2,097,510

## PRIMING MIXTURE

Willi Brün, Stratford, Conn., assignor to Remington Arms Company, Inc., a corporation of Delaware

No Drawing. Application August 3, 1935,  
Serial No. 34,637

4 Claims. (Cl. 52—4)

This invention relates to priming mixtures for small arms ammunition, and contemplates the use of a novel explosive ingredient therefor.

The lead salts of styphnic acid, particularly the normal lead salt, have acquired extensive use as the explosive ingredient of ammunition priming mixtures, but hitherto no other styphnates have been deemed suitable for this purpose. It has now been discovered that the silver styphnates, particularly normal silver styphnate of the composition  $C_6H(NO_2)_2O_2Ag_2$ , are excellent explosive ingredients for ammunition priming compositions, being in many respects superior even to normal lead styphnate. Particularly, it has been found that by the use of this silver salt it is feasible to prepare and load non-mercuric non-corrosive mixtures into centerfire cartridges in a dry condition, a result which has not hitherto been attained. Silver styphnate may be prepared by the addition of a solution of a soluble silver salt of a strong acid, such as nitric acid, to a solution of a soluble styphnate, such as magnesium styphnate. Excellent yields of the silver salt in a condition suitable for use as an ingredient of priming mixtures are secured. Typical compositions are as follows:

|                   | Per cent | Per cent      |
|-------------------|----------|---------------|
| Mercury fulminate | 10 to 35 | preferably 20 |
| Silver styphnate  | 5 to 30  | do 20         |
| Antimony sulphide | 5 to 20  | do 9          |
| Calcium silicide  | 5 to 15  | do 7          |

|                    | Per cent | Per cent     |
|--------------------|----------|--------------|
| Lead peroxide      | 3 to 10  | preferably 7 |
| Barium nitrate     | 10 to 50 | do 37        |
| Guanylnitrosamino- |          |              |
| guanyltetrazene    | 1 to 4   | do 2 5       |
| Silver styphnate   | 30 to 45 | do 38        |
| Barium nitrate     | 25 to 60 | do 39        |
| Lead peroxide      | 3 to 15  | do 5         |
| Antimony sulphide  | 2 to 20  | do 5         |
| Calcium silicide   | 2 to 20  | do 11 10     |

What is claimed is:

1. An ammunition priming composition containing a silver salt of styphnic acid.
2. An ammunition priming composition containing di-silver styphnate.
3. An ammunition priming composition containing a sensitizing ingredient, oxidizing and fuel ingredients, and a silver styphnate.
4. An ammunition priming composition substantially as follows:

|                    | Per cent | Per cent     |
|--------------------|----------|--------------|
| Guanylnitrosamino- |          |              |
| guanyltetrazene    | 1 to 4   | preferably 2 |
| Silver styphnate   | 30 to 45 | do 38        |
| Barium nitrate     | 25 to 60 | do 39 25     |
| Lead peroxide      | 3 to 15  | do 5         |
| Antimony sulphide  | 2 to 20  | do 5         |
| Calcium silicide   | 2 to 20  | do 11        |

WILLI BRÜN. 30